

# United States Patent [19]

Sugi et al.

[11] 3,925,573

[45] Dec. 9, 1975

[54] RECORDING METHOD

[75] Inventors: Ichiro Sugi; Haruo Takenaka; Toshiaki Okiyama, all of Tokyo; Teruo Kobayashi, Minami-ashigara, all of Japan

[73] Assignee: Fuji Photo Film Co., Ltd., Minami-ashigara, Japan

[22] Filed: Feb. 12, 1974

[21] Appl. No.: 441,784

Related U.S. Application Data

[62] Division of Ser. No. 214,215, Dec. 30, 1971.

[30] Foreign Application Priority Data

Dec. 30, 1970 Japan..... 45-123039

[52] U.S. Cl. .... 427/145; 8/4; 8/14; 8/69; 427/146; 427/150

[51] Int. Cl.<sup>2</sup> .... B44F 1/10; G03C 11/22

[58] Field of Search .... 8/4, 14, 69; 117/36.2, 117/36.8, 36.9, 1.7; 427/145, 146, 150

[56] References Cited

UNITED STATES PATENTS

1,642,774 9/1927 Grange ..... 117/1.7

|           |         |                      |          |
|-----------|---------|----------------------|----------|
| 2,922,690 | 1/1960  | Mueller et al. ....  | 8/21     |
| 3,148,934 | 9/1964  | Brookens et al. .... | 8/4      |
| 3,155,513 | 11/1964 | Sorenson ....        | 96/91    |
| 3,367,797 | 2/1968  | Sorenson ....        | 117/36.8 |
| 3,677,786 | 7/1972  | Hollmann et al. .... | 117/1.7  |

OTHER PUBLICATIONS

Knechi et al., *The Principles & Practice of Textile Printing*, pp. 663, 664, 1952.

Primary Examiner—Michael R. Lusignan  
Attorney, Agent, or Firm—Sughrue, Rothwell, Mion,  
Zinn & Macpeak

[57]

ABSTRACT

A recording material of a polymeric film comprising a polymeric film such as a polyester film and a layer of a bleachable dye such as a triphenylmethane type dye. The dye layer can be bleached with a writing instrument containing a bleaching agent to give a transparent clear drawing. The material is useful for overhead projection to give a clear image that is easy to see.

10 Claims, 5 Drawing Figures



FIG.1



FIG.2



FIG.3



FIG.4



FIG.5



## RECORDING METHOD

This is a division of application Ser. No. 214,215, filed Dec. 30, 1971.

This invention relates to a recording material of a polymeric film, and more specifically, to a polymeric film recording material comprising a polymeric film and a readily bleachable dye layer coated thereon.

A negative recording method wherein a non-transparent film layer is coated on a polymeric film, and then the coated film layer is removed thereby to render it transparent and perform recording is one of the feasible recording methods because of various merits such as the ease of seeing, the freedom from eye fatigue, or the usability of a coating layer having various colors. The conventional methods, however, include a method wherein a film layer coated on the polymeric film is cut off by applying a pressure to make it transparent, or by a method wherein the desired parts of the coated film layer are stripped off to make them transparent, both methods performing recording by applying an external physical force.

These recording materials, however, have the defect that letters, figures, etc., cannot be drawn freely thereon.

It has now been found that when a layer of a readily bleachable dye is coated on a polymeric film and a recording is made by using a writing instrument containing a bleaching agent, an oxidation reduction reaction (chemical reaction) occurs to bleach the dye layer, and recording is performed easily, rapidly, and freely.

Accordingly, an object of the present invention is to provide a recording material on which letters, figures, etc., can be easily drawn.

Another object of the invention is to provide a negative material by coating a dye layer readily removable by a remover on a polymeric film and then bleaching the dye layer with a writing instrument containing the remover utilizing an oxidation reduction reaction (chemical reaction).

The invention will be described with reference to the accompanying drawings in which:

FIG. 1 is a sectional view of one example of the recording material of the invention;

FIG. 2 is a sectional view of one example of the recording material of the invention in which recording has been made with a writing instrument containing a bleaching agent;

FIG. 3 is a sectional view of one example of the recording material of the invention in which recording has been made with a writing instrument containing a bleaching agent and a dye;

FIG. 4 is a sectional view of another example of the recording material of the invention; and

FIG. 5 is a sectional view of the recording material of the invention in which three colors are combined.

In these drawings, the reference numeral 1 designates a polymeric film, and a colored film layer which is readily bleachable with a bleaching agent is shown at 2, 2', or 2''. The reference numeral 3 represents a writing instrument containing a bleaching agent. The bleached part of the film layer obtained by the writing instrument 3 is designated at 4. The reference numeral 5 shows a part on which recording has been performed in a color different from that of the coated layer upon bleaching the film layer with the writing instrument 3.

FIG. 5 shows that by combining three primary colors (yellow, magenta and cyan), various color phases can be selected.

The dyes that can be used in the dye layer of the invention must be readily bleached by an oxidation reduction reaction. Examples of such dyes that can be used in the invention are dyes expressed by the following general formulae I, II and III. At least one of such dyes is dissolved in a solvent to be described, and the resultant solution is coated on a polymeric film to form a dye layer. In order to improve adhesion between the polymeric film and the dye layer, a binder to be described may be added to the solution of the dye layer.

## General Formula I



wherein  $R_1$  and  $R_2$  may be the same or different and each represents a hydrogen atom, a lower alkyl group having 1 to 5 carbon atoms, an hydroxyalkyl group, a sulfoalkyl group, aryl group, or an aralkyl group;  $R_3$  and  $R_4$  are



wherein  $R'_1$  and  $R'_2$  are the same as  $R_1$  and  $R_2$ , a hydrogen atom, a hydroxyl group, a halogen atom, a lower alkyl group having 1 to 5 carbon atoms, an alkoxy group, a carboxyl group, or a sulfone group, and may be the same or different; phenylene nucleus 1 may be substituted by an alkoxy group, a halogen atom, or a lower alkyl group having 1 to 5 carbon atoms,  $n$  is from 1 to 3; and  $X$  is an anion or an anion of an intramolecular salt.

The dyes expressed by the general formula 1 are triphenylmethane dyes. Since they are colored yellow, orange, red, violet, blue, and green, it is possible to choose various colors for use as a dye layer. Furthermore, since these dyes are soluble in a variety of solvents such as alcohols or others to be described, the dye layer becomes fast-drying. They are also readily bleached with a bleaching agent to be described, and the color does not return to the original one. Examples of the dyes of formula 1 are listed below. The colors indicated are those obtained by coloring.

## I Examples of dyes

## Structure



Color Reference Yellow  
Berichte 37, 601



Color Reference bluish green  
Am. Chem., 206, 96



Color violet



Color Reference red  
C.I. 42510



Color Reference violet  
C.I. 42535



Color Reference blue  
C.I. 42140



Color Reference bluish green  
C.I. 42000

-continued

I Examples  
of dyes

## Structure

|    |  |                            |                                          |
|----|--|----------------------------|------------------------------------------|
| 7  |  | Color Reference            | bluish green                             |
|    |  |                            | Japanese Patent Publication No. 18637/65 |
| 8  |  | Color Reference            | bluish violet                            |
|    |  | C.I.                       | 43525                                    |
| 9  |  | Color Reference            | blue                                     |
|    |  | Disulfone compound of C.I. | 42755                                    |
| 10 |  | Color Reference            | blue                                     |
|    |  | C.I.                       | 42655                                    |
| 11 |  | Color Reference            | blue                                     |
|    |  | C.I.                       | 42655                                    |
| 12 |  | Color Reference            | blue                                     |
|    |  | C.I.                       | 42705                                    |

-continued

## I Examples of dyes

## Structure

13

Color  
Reference red violet  
C.I.

43565

14

Color  
Reference red violet  
C.I.

43570

15

Color  
Reference green  
C.I.

42010

16

Color  
Reference green  
Journal of Chemical  
Society, 41, 193 and  
Berichte 15, 237

## General formula II

where R<sub>5</sub> is H, lower alkyl having 1 to 5 carbon atoms, aryl group, or COOM, M being hydrogen atom, alkali

meta, ammonium, or lower alkyl group having 1 to 5 carbon atoms; R<sub>6</sub> is hydrogen atom, hydroxyl group, SO<sub>3</sub>M, M being hydrogen atom, alkali metal, or ammonium, alkoxy group, halogen atom, or dialkylamino group; and R<sub>7</sub> is hydrogen atom, lower alkyl group having 1 to 5 carbon atoms, or aryl group.

General formula II represents pyrazolobenzylidene type dyes. They are yellow to orange, soluble in the below-mentioned solvents such as alcohols, and readily bleached with bleaching agents to be described, the colors not returning to the originals.

Examples of dyes of formula II are as follows:

## II Examples of dye

## Structure

## Color

17



Yellow

-continued

## II Examples of dye

## Structure

## Color

18



Light yellow

19



Yellow

20



Yellow

21



Yellow

22



Orange red

23



Yellow

-continued

## II Examples of dye

## Structure

## Color

24



Yellow orange

## General formula III



wherein  $R_8$  is lower alkyl group having 1 to 5 carbon atoms,  $R_9$  is lower alkyl, substituted alkyl group, or aryl group;  $R_{10}$  is hydrogen atom or methyl;  $R_{11}$  is hydrogen atom, halogen group and carboxymethyl group; and  $X$  is an anion.

The general formula III represents indolinostyryl type dyes which are red to violet, soluble in solvents such as alcohols, and readily bleached with bleaching agents to be described, the colors not returning to the originals.

Examples of dyes of formula III include:

## III Examples of dyes

## Structure

Color Reference pink C.I.

48015

25



26



Color Reference pink C.I.

48013

27



Color Reference red violet C.I.

48020

28



Color Reference red C.I.

48013

-continued

## III Examples of dyes

## Structure

29

Color violet  
Reference C.I.

48030

30

Color violet  
Reference C.I.

48025

## General formula IV



wherein  $R_1$  and  $R_2$  are hydrogen atom, alkyl group of not more than 5 carbon atoms and may be the same or different and  $X$  is an acid residue.

| Examples of dyes | $R_1$       | $R_2$  | Color |
|------------------|-------------|--------|-------|
| 35               | H           | H      | blue  |
| 36               | $CH_3$      | H      | blue  |
| 37               | $CH_3$      | $CH_3$ | blue  |
| 38               | $C_6H_{11}$ | H      | blue  |

wherein  $R_1$  and  $R_2$  are lower alkyl group of not more than 5 carbon atoms;  $R_3$  and  $R_4$  are hydrogen atom, lower alkyl having 1 to 5 carbon atoms, or aralkyl group; and  $X$  is an acid residue.

Examples of the solvent used for dissolving the dyes I, II, III, IV, and V above include lower alcohols such as methanol, ethanol or propanol, or other readily evapo-

| Examples of dyes | $R_1$    | $R_2$    | $R_3$    | $R_4$    | Color |
|------------------|----------|----------|----------|----------|-------|
| 31               | $C_2H_5$ | $C_2H_5$ | $CH_3$   | H        | black |
| 32               | $C_2H_5$ | $C_2H_5$ | $C_2H_5$ | $C_2H_5$ | green |
| 33               | $C_2H_5$ | $C_2H_5$ | $-CH_2-$ | H        | black |
| 34               | $C_2H_5$ | $C_2H_5$ | $-CH_2-$ | $-CH_2-$ | green |

## General formula V



rating and drying organic solvents such as acetone, or dioxane. Mixtures of water with the organic solvents can also be used.

A binder may be used for inclusion in the coated film layer in order to improve adhesion between the polymeric film and the film layer. Examples of the binder include tragacanth rubber, British rubber, sodium alginate, polyvinyl alcohol, and carboxymethyl cellulose which are used mainly as aqueous solutions, and syn-

thetic resins such as a polycondensate of cresol, salicylic acid or oxyphenylacetic acid with formaldehyde, a polymer of acrylic acid, methacrylic acid, or of styrenecarboxylic acid, a copolymer of vinyl chloride and acrylic acid, a copolymer of vinyl chloride and maleic anhydride, a copolymer of acrylonitrile and styrenecarboxylic acid, a copolymer of vinyl acetate and maleic anhydride, a copolymer of styrene and maleic anhydride, a copolymer of vinyl butyl ether and styrenesulfonic acid, cellulose acetate phthalic acid ester, or cellulose acetate maleic acid ester which are used mainly as alcohol, acetone, or dioxane solutions. The amount of the binder used in the invention is adequately 50 to 500% based on the weight of the dye. The use of more than 500% causes difficulty of bleaching.

The solution containing these dyes or binders is coated on a film of a polymer such as polyethylene terephthalate, cellulose esters, polycarbonate, vinyl polymers or polystyrene, to thereby form a dye layer.

As the bleaching agent for the dye layer, addition

5  
10

products of sulfites and/or bisulfites with formaldehyde are used (the salts here are sodium, potassium and ammonium salts). Examples of other useful bleaching agents include sodium bisulfite, hydrosulfite, an addition product of hydrosulfite with formaldehyde, sodium sulfoxylate formaldehyde ( $\text{NaHSO}_2\text{CH}_2\text{O}\cdot 2\text{H}_2\text{O}$ ) sulfur dioxide gas, sodium sulfide, thiourea dioxide, hydrazines such as hydrazine hydrate, or phenyl hydrazine, and amines such as ethanolamine or butylamine.

A solution of the bleaching agent in water or an organic solvent such as alcohols, e.g. methanol or ethanol, and ketones such as acetone or methyl ethyl ketone is put in a writing instrument such as "sign pens" or "magic pens".

15 If desired, a dye which is difficult to bleach with said bleaching agent may be incorporated in the bleaching agent. By this, it is possible to form a color of the dye incorporated in the writing instrument on the bleached part of the coated dye layer. Examples of dyes which are difficult to bleach are:



Color yellow, C.I. 49000.



Color red

C.I. 29160



Color blue

C.I. 74180

(d)



Color violet; C.I.

60730



The recording material so obtained finds a variety of applications such as overhead projection or drafting. When it is used as a film for overhead projection, it is easy to see without causing eye fatigue. Moreover, various colors can be chosen for use in background, that is, a coated film layer. Using this material, recording can be performed freely and rapidly, and a negative can be obtained with simplicity.

The invention will be described specifically by the following Examples.

#### EXAMPLE 1

Dye No. 2A (3 g) was dissolved in 100 g of methanol to prepare a dye solution (solution A). On the other hand, 5 g of a copolymer of vinyl acetate and maleic anhydride was dissolved in 100 g of ethyl alcohol to prepare a binder solution (solution B). These solutions A and B were mixed with each other, and the mixed solution was coated on a 100  $\mu$  thick film of cellulose triacetate, and dried to form a blue film.

Separately, 5 g of ammonium sulfite was dissolved in 50 g of water and 50 g of methanol to form a bleaching agent solution in a sign pen receptacle. Writing was made on the blue film using this sign pen. A colorless transparent line drawing was obtained. When it was projected with an overhead projector, a clear image was obtained which did not give fatigue to the eyes.

#### EXAMPLE 2

Dye No. 2B (5 g) was dissolved in 50 g of methanol and 50 g of methylene dichloride. To the resultant solution was added a bleaching agent solution of 10 g of a polycondensate of salicylic acid with formaldehyde in 100 g of ethanol. The mixed solution was coated on a 75  $\mu$  thick polyester film, and dried to form a violet film. Writing was made on the film obtained, using a 5% aqueous solution of sodium sulfite (or 10% ethanalamine methanol solution or 10% hydrazine hydrate methanol solution). A colorless transparent line drawing was rapidly obtained.

#### EXAMPLE 3

Example 2 was repeated except that dye (a) (yellow dye which is difficult to bleach; dye table No. 49000) was put into the bleaching agent solution in an amount of 1% by weight. A yellow line drawing was obtained in the resulting violet film.

#### EXAMPLE 4

Example 1 was repeated except using each of dyes Nos. 1 and 3 to 34, to obtain films of the colors indicated hereinabove. When writing was made on each of the film using the bleaching agent solution, a colorless transparent line drawing was obtained, and the film permitted the projection of an image that could be easily seen.

#### EXAMPLE 5

Dye No. 35 (2 g) was dissolved in 100g of chloroform. On the other hand, 5 g of a copolymer of vinyl butyl ether and styrenesulfonic acid was dissolved in 100 g of ethanol. The resultant solutions were mixed with each other. Subsequently, the same procedure as set forth in Example 2 was repeated to form a blue film. A colorless and transparent line drawing was rapidly obtained using a bleaching agent solution.

The same results were obtained with dyes Nos. 36 to 38.

#### EXAMPLE 6

A 1% aqueous solution of dye No. 6 (2.5 g) was mixed with 2 g of a 10% aqueous solution of gelatin, and the mixed solution was coated on a transparent 75  $\mu$  thick polyester film to form a cyan colored layer. When writing was made on the film using a 20% methanol solution of ethanalamine, a colorless transparent line drawing was obtained rapidly.

On the other hand, 4 g of a 1% aqueous solution of dye No. 20 and 3 g of a 10% aqueous solution of gelatin were similarly coated on another polyester film to form a yellow layer. On the back of this film were coated 1.5 g of a 1% aqueous solution of dye No. 26 and 2 g of a 10% aqueous solution of gelatin to form a magenta layer.

Writing was made with a 10% aqueous solution of sodium sulfite on suitable places of these front and back surfaces. The written parts were bleached. FIG. 5 shows the superposition of these two films.

What is claimed is:

1. A recording method which comprises drawing on a coated film with a writing instrument having a bleaching agent, said film being transparent and having at least one layer of a dye bleachable by said bleaching agent coated thereon, said bleaching agent bleaching said dye to cause it to become transparent.

2. The recording method of claim 1, wherein said bleaching agent in said writing instrument includes a dye which is resistant to bleaching whereby the areas of said layer of dye bleached by said bleaching agent are colored by the bleach-resistant dye.

3. A method of recording on a transparent polymeric film for overhead projection comprising drawing on a layer of a bleachable dye coated on the transparent polymeric films with a writing instrument which has a bleaching agent therein, said bleaching agent of said writing instrument bleaching said bleachable dye such that the recording is obtained.

4. The recording method of claim 3, wherein said layer of said dye contains a binder which improves the adhesion between said transparent polymeric film and said layer of said bleachable dye.

5. The recording method of claim 3, wherein a dye which is resistant to bleaching with said bleaching

agent is incorporated in said bleaching agent in said writing instrument, said dye thereby coloring the areas bleached by said bleaching agent.

6. The recording method of claim 3, wherein said bleachable dye is bleachable by an oxidation-reduction reaction of said dye and said bleaching agent.

7. The recording method of claim 3, wherein said bleachable dye is a member selected from the group of dyes listed below as represented by Formulae I, II, III, IV and V:



wherein  $R_1$  and  $R_2$  may be the same or different and each represents a hydrogen atom, a lower alkyl group having 1 to 5 carbon atoms, a hydroxyalkyl group, a sulfoalkyl group, an aryl group or an aralkyl group;  $R_3$  and  $R_4$  are



wherein  $R'_1$  and  $R'_2$  are the same as  $R_1$  and  $R_2$ , a hydrogen atom, a hydroxyl group, a halogen atom, a lower alkyl group having 1 to 5 carbon atoms, an alkoxy group, a carboxyl group, or a sulfone group and may be the same or different; phenylene nucleus 1 may be substituted by an alkoxy group, a halogen atom, or a lower alkyl group having 1 to 5 carbon atoms,  $n$  is from 1 to 3; and  $X$  is an anion or an anion of an intramolecular salt;

50

wherein  $R_1$  and  $R_2$  are lower alkyl group or not more than 5 carbon atoms;  $R_3$  and  $R_4$  are hydrogen atom, lower alkyl group having 1 to 5 carbon atoms, or aralkyl group; and  $X$  is an acid residue;



wherein  $R_1$  and  $R_2$  may be the same or different and each represents an alkyl group of not more than 5 carbon atoms, and X is an acid residue.

8. The recording method of claim 3, wherein said bleaching agent is selected from the group consisting of addition products of sulfites, bisulfites, or both sulfites and bisulfites with formaldehyde, sodium bisulfite, hydrosulfite, an addition product of hydrosulfite with formaldehyde, sodium sulfoxylate formaldehyde, sulfur dioxide gas, sodium sulfide, thiourea dioxide, hydroazines, and amines.

9. The recording method of claim 4, wherein said binder is a member selected from the group consisting of tragacanth rubber, British rubber, sodium alginate, polyvinyl alcohol, carboxymethyl cellulose, polycon-

densates of a member selected from the group consisting of cresol, salicylic acid and oxyphenylacetic acid with formaldehyde, acrylic acid polymers, methacrylic acid polymers, styrene carboxylic acid polymers, a copolymer of vinyl chloride and acrylic acid, a copolymer of vinyl chloride and maleic anhydride, a copolymer of acrylonitrile and styrene carboxylic acid, a copolymer of vinyl acetate and maleic anhydride, a copolymer of styrene and maleic anhydride, a copolymer of vinyl butyl ether and styrene sulfonic acid, cellulose acetate phthalic acid ester, and cellulose acetate maleic acid ester.

10. The recording method of claim 4, wherein the amount of said binder ranges from 50 to 500 percent by weight based on the amount of said dye.

\* \* \* \* \*